

# UNITED STATES PATENT OFFICE.

RAYMOND F. BACON, OF PITTSBURGH, PENNSYLVANIA, ASSIGNOR TO METALS RECOVERY COMPANY, OF NEW YORK, N. Y., A CORPORATION OF MAINE.

## CONCENTRATION OF ORES.

1,197,590.

Specification of Letters Patent. Patented Sept. 12, 1916.

No Drawing.

Application filed November 10, 1915. Serial No. 60,697.

To all whom it may concern:

Be it known that I, RAYMOND F. BACON, a citizen of the United States, residing at Pittsburgh, Allegheny county, State of Pennsylvania, have invented certain new and useful Improvements in Concentration of Ores; and I do hereby declare the following to be a full, clear, and exact description of the invention, such as will enable others skilled in the art to which it appertains to make and use the same.

This invention relates to the concentration of ores and to the separation of metal constituents thereof from each other and from associated gangue, by a procedure which involves a fractional separation of the metal constituents and conversion thereof into a form suitable for flotation, and by a subsequent flotation treatment.

In the common flotation processes of concentrating low grade sulfid ores, the process involves an indiscriminate separation of sulfid from gangue. Where the sulfid particles are themselves superficially oxidized or coated with an oxid film, it has been common practice to effect the flotation in the presence of an acid which will dissolve and thus remove such oxid films and leave the sulfid particles suitable for flotation. This solution of oxid constituents, however, results in a loss of metal values, which can only be recovered by a subsequent treatment, and which are often present in such dilute solution as to make recovery impracticable.

It has heretofore been proposed to effect a selective separation of sulfid ores by first subjecting the ores to a partial roast to convert some of the constituents into a form unsuited to flotation and then floating the unchanged sulfids from the thus changed constituents. Such proposals are open to the objection that a clean separation is not possible with many ores since it is difficult to completely convert certain sulfids without partially converting them all, and to the extent that those sulfids are converted which it is desired to retain as sulfids, their separation is prevented. Oxidized constituents remain with the tailings and are not separated. Moreover, in many ores the sulfids are so intimately blended that it is impossible to effect a clean separation of said non-sulfids from each other, or to effect a selec-

tive oxidation or deadening of said constituents only.

It has also been proposed to convert oxid ores into sulfids by treatment with hydrogen sulfid or soluble sulfids, and by thereafter subjecting the ore to flotation; but such procedures also involve an indiscriminate separation of all sulfids formed from the gangue. Where the oxid or other non-sulfid constituents are present intimately blended with each other and with the gangue, the sulfidized ore retains the constituents in a corresponding state of combination.

It has also been proposed to separate oxidized lead and zinc compounds in suspension in the presence of an acid by treatment with sulfureted hydrogen or a soluble sulfid, thereby coating only the lead with a layer of sulfid without converting the oxidized zinc into sulfid, the zinc oxid not being affected by the sulfid in an acid solution; the thus partially sulfidized ore being subsequently subjected to flotation. With many ores, such a proposal is not practicable because of the intimate blending of the lead and zinc with each other and with the gangue, even in a finely crushed condition. Where the lead and zinc are thus blended, the particles will remain physically combined even after partial sulfidization and a clear separation will be thus precluded. Moreover, to the extent that the gangue is physically attached to the oxid or sulfid particles, it will either be removed with such particles or will prevent the desired separation thereof.

All of the various procedures referred to above involve a preliminary crushing to effect a physical separation of the gangue from the ore. Where the ores are of such a nature that such physical separation cannot be effected by crushing, the separation is to that extent prevented and prejudiced. Similarly, the proposals to effect selective separation of different sulfid constituents from each other or from oxid constituents are subject to the limitation that where these constituents are intimately combined together in the same finely divided particles, their separation is not practicable for the reason that the treated particles still retain such constituents in a similar state of combination.

The process of the present invention is

an improvement on such prior processes and proposals, overcoming many of the disadvantages indicated above, and enabling in addition new and improved results to be obtained. As distinguished 5 from such indiscriminate separations of sulfid constituents from gangue, as have been referred to, the process of the present invention involves a selective or fractional 10 separation of metal constituents from each other and from the gangue which will be more clear and sharp, and which can be applied to ores incapable of satisfactory concentration by methods heretofore proposed. 15 While all of the proposals referred to above depend primarily upon the physical separation of the ore from the gangue and of different-ore constituents from each other, the process of the present invention enables a 20 separation of metal constituents from each other and from the gangue to be effected where such physical separation by crushing 25 is not possible.

The process of the present invention comprises a preliminary treatment of the ores 25 to convert part or all of the metal constituents into a soluble form, where these constituents are not already soluble, and a subsequent treatment of the soluble constituents with a suitable acid to effect solution thereof. Subsequently the dissolved metal constituents are fractionally precipitated within the pulp as sulfids, and finally the precipitated sulfids are separated from the 35 ore pulp by flotation.

The solution and precipitation processes of obtaining metals from their ores, heretofore practised, involve dissolving the metal values, filtering the dissolved values 40 from the ore pulp and washing and draining the ore pulp to complete the separation of the dissolved constituents. Such processes are practicable with relatively concentrated ores, but with low grade ores having 45 large amounts of gangue material, the separation of the dissolved constituents from the ore pulp by filtering and by subsequent washing is a slow and imperfect procedure. Where silicate ores are treated, 50 more or less silicic acid is often set free, of a more or less gelatinous nature, which further impedes the filtration of the ore pulp. When the solutions are finally obtained, they are usually more or less dilute, 55 requiring the handling of large volumes of liquid from which the metal values must be precipitated after preliminary purification. As distinguished from such solution and precipitation processes where filtration followed 60 by precipitation and a second filtration is necessary, the process of the present invention comprises dissolving and precipitating the metal values within the pulp as sulfids, and effecting the separation of the thus precipitated sulfids by flotation meth-

ods, whereby the disadvantages of the old solution and precipitation processes are overcome while the advantages of such processes are largely retained. Thus it is possible to effect substantially complete 70 solution of certain metal constituents, or of all metal constituents, from the gangue even where the crushed ore particles contain the gangue intimately blended with the ore. The process of the present invention further comprises a fractional precipitation and separation by flotation of the dissolved metal values, whereby the metal constituents can be fractionally separated from each other. 75

The ores which can be treated according to the present invention may be either of a sulfid or of an oxid or other non-sulfid nature. The process is of more or less general application to ores containing different 80 metal constituents, particularly metal constituents which form acid insoluble sulfids. Where the ores are already of an oxidized nature, they can be treated without further preliminary preparation than a suitable 85 crushing. This crushing, moreover, need not be as fine and complete as has heretofore been necessary with flotation processes inasmuch as, by the present process, the metal constituents can be effectively separated without being entirely separated physically 90 from associated gangue. 95

In treating sulfid ores, a preliminary roast, either partial or complete, is often necessary or advantageous. Thus with zinc 100 blend ores containing lead, the lead and zinc sulfids are so intimately combined and blended with each other that it is impossible to effect physical separation by any crushing procedure. In order to effect separation of such ores, it is necessary to dissolve the zinc and thus separate it from the lead. Where the zinc sulfid is soluble directly in dilute acid, it can be thus dissolved without 105 preliminarily roasting but it may, however, be more advantageous to subject the ore to a preliminary roast and thus loosen the texture of the ore particles so that they can be more readily extracted and dissolved. 110

The invention will be described more in 115 detail in connection with the treatment of certain specific ores, from which the nature and advantages of the invention will more clearly appear. It will be understood, however, that the invention is of more general 120 application and that it is illustrated by, but is not limited to, these specific illustrations of its application.

In treating copper sulfid ores containing 125 iron pyrites, or in treating mixed copper and iron sulfid ores such as chalcopyrite, with which iron pyrites is usually present, the ore is subjected to a preliminary roast at a red heat or at a suitable temperature to decompose the iron sulfid and leave the copper in 130

the form of sulfid. By such treatment, however, more or less copper may also be oxidized, and the copper originally present in an oxidized state will also be present after the recasting in a soluble form. More or less silver, lead, zinc, etc., may also be present. After the preliminary roast, the ore is treated with dilute sulfuric acid to dissolve the iron and other soluble constituents, including the soluble copper oxid and other soluble salts. Hydrogen sulfid is then passed into the ore pulp to precipitate dissolved copper as sulfid together with other metal sulfids insoluble in the dilute acid solution, without, however, precipitating zinc or iron as sulfids or other acid-soluble sulfids. Upon then subjecting the ore pulp to a flotation treatment, the copper sulfid can be floated off leaving the iron and other soluble constituents in solution. If zinc is present, or if a further separation by flotation of dissolved constituents is desired, this can be effected in a manner more fully hereinafter described.

Where copper ores are already in an oxidized state, the preliminary roast is not necessary, but the separation can be effected by solution and fractional precipitation in the manner above described. Where the iron is present in considerable amounts, the resulting iron sulfate solution can be separated from the pulp and used for extracting fresh amounts of ore.

Where the ore contains copper and zinc together, in the form of oxids, both metals can be dissolved with dilute sulfuric acid or with other suitable solvent, and the copper precipitated as sulfid by treatment with hydrogen sulfid in the presence of a suitable excess of acid. After subjecting the pulp to flotation and thereby separating the copper, the zinc can be precipitated as sulfid by neutralizing the excess acid and by treatment with a suitable sulfid such as an alkaline sulfid or an alkali or alkaline earth sulfhydrate, and the precipitated zinc sulfid can be subsequently separated by a further flotation treatment.

In the treatment of the pulp containing both copper and zinc in solution, with hydrogen sulfid, zinc sulfid may be temporarily precipitated in dilute solutions, but this can be prevented by a suitable amount of acid. Also the precipitated zinc sulfid will itself react with dissolved copper to form copper sulfid, the zinc again going into solution.

In treating ores containing copper and nickel, in the form of sulfids, together with iron pyrites, the ore can be treated directly with sulfuric acid to dissolve the nickel or the nickel and copper, to the extent that the copper is soluble, and the copper can be then precipitated in the presence of a suitable excess of acid, without precipitating the nickel sulfid, by treatment with hydrogen sulfid. The nickel can be subsequently precipitated

as sulfid by neutralizing the acid and by treatment with the soluble sulfid, after which the precipitated nickel sulfid can be itself recovered by a further flotation treatment.

In treating an ore containing lead, silver, and zinc, in the form of sulfids, the ore can be decomposed with the evolution of hydrogen sulfid by treatment with hydrochloric acid and an oxidizing agent, or the ore may be decomposed by a chloridizing roast. With oxid ores the chlorids can be formed directly without evolution of such gas. The chlorids of silver and lead are relatively insoluble, although more soluble than the corresponding sulfids. By treating the resulting solution containing zinc chlorid and small amounts of lead and silver chlorids, there being also silver and lead chlorids in suspension, with hydrogen sulfid in the presence of a suitable excess of the acid the dissolved lead and silver will be precipitated as sulfids and the suspended chlorids will also be converted into sulfids superficially or completely by sufficiently prolonging the hydrogen sulfid treatment. The lead and silver sulfids can then be floated from the gangue leaving the zinc in solution. The zinc will be recovered by a subsequent treatment in the manner above indicated.

In treating the zinc blende ores containing lead together with iron pyrites and more or less copper sulfid, it is advantageous to subject the ore to a preliminary roast to convert the ore more or less completely into an oxidized or sulfatized condition. The ore should be, of course, in a finely ground state, although it is not necessary that the ore should be as finely crushed as has heretofore been considered necessary. The ore can be roasted only to a dull red heat for a few minutes to loosen the texture of the ore and to decompose iron pyrites together with part of the other sulfids, or the ore can be completely oxidized or sulfatized by prolonging the roasting operation or by carrying out this operation at higher temperatures.

The resulting ore is treated with sulfuric acid to dissolve the iron together with other soluble constituents. If the roast is such as to convert the sulfids into sulfates, the lead will remain as sulfate and will not go into solution. The zinc, however, will be dissolved together with more or less copper, if the copper has been made soluble. Upon treating the resulting acid pulp with hydrogen sulfid the copper will be precipitated as sulfid and the lead sulfate, although relatively insoluble will, nevertheless, be converted superficially into sulfid by prolonging the hydrogen sulfid treatment, since lead sulfid is even less soluble than lead sulfate. Accordingly, upon subjecting the ore pulp to flotation the copper and lead sulfids together with sulfid coated lead sulfate where

the lead sulfate has not been completely sulfidized, will be floated and separated from the ore pulp while the zinc and iron will remain in solution. The zinc can be subsequently recovered by precipitation as sulfid and by another flotation treatment in the manner already described.

Instead of using hydrogen sulfid, other soluble sulfids can be used in a similar manner, since, in the presence of an excess of acid such sulfids will be hydrolyzed into hydrogen sulfid. Accordingly, I consider such soluble sulfids in the presence of a suitable excess of acid as the equivalents of hydrogen sulfid for purposes of the present invention.

In precipitating zinc or nickel, after the acid insoluble sulfids have been precipitated and removed, the excess acid should be neutralized. By then treating the ore pulp with an alkali sulfid such as sodium sulfid or with an alkaline earth sulfid or sulfhydride, such as calcium sulfhydride, the zinc or nickel can then be precipitated and its flotation thereafter effected. After the precipitation of the zinc, any excess hydrogen sulfid or soluble sulfid should advantageously be neutralized and the pulp rendered faintly acid to promote the flotation process.

Instead of using sulfuric acid, sulfur dioxid or mixtures of sulfur dioxid with sulfur trioxid can be used in a more or less similar manner. By using sulfur dioxid as the extracting agent for forming the solutions of the metals within the pulp, and by subsequently treating with hydrogen sulfid, not only will the acid insoluble metal sulfids be precipitated, but colloidal sulfur will also be formed.

In my companion application Serial No. 36,698, filed June 28, 1915, I have described and claimed the treatment of non-sulfid ores, either simultaneously or successively, with sulfur dioxid and hydrogen sulfid, and thereby effecting a sulfidizing of the ore and the formation of colloidal sulfur within the ore pulp. In said companion application, I have also described and claimed the fractional or selective separation of metal constituents from each other by such colloidal sulfur process. The claims of said application, however, are limited to a procedure wherein such colloidal sulfur is formed and made use of for effecting separation; while in the present application the claims are drawn generically to the fractional or selective separation by the use of any suitable acid, and specifically to the use of sulfuric acid, as distinguished from the use of sulfur dioxid.

In separating the precipitated sulfids from the ore pulp and gangue by flotation, the pulp may be subjected to aeration, with agitation, and the flotation thereby effected,

or a small amount of oil can be beaten into the pulp together with the air, and a froth thus obtained. In either case, the flotation is materially improved by the presence of the precipitated sulfids which are of a more or less colloidal nature than the naturally occurring sulfid constituents of the ore.

From the above description it will be seen that the invention is of more or less general application, both to the treatment of completely oxidized ores and to the treatment of ores only partially oxidized. In all cases the procedure involves a preliminary solution of acid soluble metal constituents to form a preliminary solution thereof within the ore pulp, and the subsequent fractional precipitation of acid insoluble sulfids within the pulp by treatment with hydrogen sulfid or other soluble sulfid in the presence of a suitable excess of acid. Inasmuch as hydrogen sulfid is readily obtainable from sulfid ores by a reducing roast, or from sulfur dioxid by heating with a suitable reducing gas; and inasmuch as sulfuric acid can also be readily obtainable from smelter fumes by oxidation; it will be seen that the reagents employed are simple and readily produced in amounts necessary for commercial operations, from the sulfid ores themselves.

It will also be seen that the process is capable of many different applications in the art, and accordingly that many variations and modifications can be made in the invention as described, without departing from its spirit and scope, as set forth in the accompanying claims.

What I claim is:

1. The method of effecting the separation of metal constituents forming acid soluble and acid insoluble sulfids from each other and from associated gangue, which comprises dissolving the acid soluble constituents of the ore with an acid and thereby forming a solution of the same in the presence of the gangue, thereafter effecting a fractional precipitation of metal constituents forming acid insoluble sulfids from those forming acid soluble sulfids by treatment with hydrogen sulfid in the presence of a suitable excess of acid, and finally subjecting the resulting mixture to a flotation treatment; substantially as described.

2. The method of effecting the separation of metal constituents forming acid soluble and acid insoluble sulfids from each other and from associated gangue, which comprises dissolving the acid soluble constituents of the ore with an acid and thereby forming a solution of the same in the presence of the gangue, thereafter effecting a fractional precipitation of metal constituents forming acid insoluble sulfids from those forming acid soluble sulfids by treatment with hydrogen sulfid in the presence of a suitable excess of acid, subjecting the

resulting mixture to a flotation treatment, subsequently precipitating as sulfids metal constituents forming water insoluble sulfids by neutralizing the excess acid and treating with a suitable sulfid, and finally subjecting the mixture to a further flotation treatment; substantially as described.

3. The method of effecting the separation of copper from metals forming acid soluble sulfids and from associated gangue, which comprises dissolving the acid soluble copper and other metal constituents of the ore with an acid and thereby forming a solution of the same in the presence of the gangue, thereafter effecting a fractional precipitation of the copper as sulfid by treatment with hydrogen sulfid in the presence of a suitable excess of acid; and finally subjecting the resulting mixture to a flotation treatment; substantially as described.

4. The method of effecting the separation of zinc from metals forming acid insoluble sulfids and from associated gangue, which comprises dissolving the zinc and other acid soluble metal constituents of the ore with an acid and thereby forming a solution of the same in the presence of the gangue, thereafter effecting a fractional precipitation of the metal constituents forming acid insoluble sulfids from the zinc by treatment with hydrogen sulfid in the presence of a suitable excess of acid, subjecting the resulting mixture to a flotation treatment, subsequently precipitating the zinc as sulfid by neutralizing the excess acid and treating with a suitable sulfid; and finally separating the zinc sulfid by a further flotation treatment; substantially as described.

5. The method of effecting the separation of sulfid ores containing iron pyrites together with other metal sulfids, which comprises subjecting such ore to a preliminary partial roast and thereby converting the iron pyrites, together with part of the other metal constituents, into an acid soluble form, dissolving such acid soluble constituents of the ore with an acid and thereby forming a solution of the same in the presence of the gangue and from the acid insoluble metal constituents, thereafter effecting a fractional precipitation of metal constituents forming acid insoluble sulfids, as sulfids without precipitating the iron, by treatment with hydrogen sulfid in the presence of a suitable excess of acid, and finally subjecting the resulting mixture to a flotation treatment; substantially as described.

6. The method of effecting the separation of lead and zinc from each other and from associated gangue in sulfid ores, which comprises roasting the ore to convert the zinc into a soluble form, dissolving the zinc and other acid soluble constituents with an acid and thereby forming a solution of the same in the presence of the gangue and from the

acid insoluble constituents, thereafter effecting a fractional precipitation and conversion of the lead, and other metal constituents forming acid insoluble sulfids, into sulfids by treatment with hydrogen sulfid in the presence of a suitable excess of acid, subjecting the resulting mixture to a flotation treatment, subsequently precipitating the zinc as sulfid, and again subjecting the mixture to a flotation treatment; substantially as described.

7. The method of effecting the separation of metal constituents forming acid soluble and acid insoluble constituents from each other and from associated gangue, which comprises dissolving the acid soluble constituents of the ore with dilute sulfuric acid and thereby forming a solution of the same in the presence of the gangue, thereafter effecting a fractional precipitation of metal constituents forming acid insoluble sulfids from those forming acid soluble sulfids by treatment with hydrogen sulfid in the presence of a suitable excess of sulfuric acid, and finally subjecting the resulting mixture to a flotation treatment; substantially as described.

8. The method of effecting the separation of zinc from metals forming acid insoluble sulfids and from associated gangue, which comprises dissolving the zinc and other acid soluble metal constituents of the ore with sulfuric acid and thereby forming a solution of the same in the presence of the gangue, thereafter effecting a fractional precipitation of the metal constituents forming acid insoluble sulfids from the zinc by treatment with hydrogen sulfid in the presence of a suitable excess of sulfuric acid, subjecting the resulting mixture to a flotation treatment, subsequently precipitating the zinc as sulfid by neutralizing the excess acid and treating with a suitable sulfid; and finally separating the zinc sulfid by a further flotation treatment; substantially as described.

9. The method of effecting the separation of lead and zinc from each other and from associated gangue in sulfid ores, which comprises subjecting the ore to a sulfatizing roast, dissolving the zinc and other acid soluble constituents with sulfuric acid and thereby forming a solution of the same in the presence of the gangue and from the insoluble constituents, thereafter effecting a fractional precipitation and conversion of the lead, and other metal constituents forming acid insoluble sulfids, into sulfids, by treatment with hydrogen sulfid in the presence of a suitable excess of acid until the lead sulfate has been sufficiently sulfidized to enable its flotation, and finally subjecting the resulting mixture to a flotation treatment; substantially as described.

10. The method of effecting the separa-

tion of lead and copper from zinc and from associated gangue in sulfid ore containing iron pyrites, which comprises roasting the ore to convert the iron pyrites together with more or less of the other metal constituents, into an acid soluble form, dissolving such acid soluble constituents of the ore with an acid and thereby forming a solution of the same in the presence of the gangue and from the acid insoluble metal constituents, thereafter effecting a fractional precipitation and conversion of

metal constituents forming acid insoluble sulfids, into sulfids, without precipitating iron and zinc sulfids, by treatment with 15 hydrogen sulfid in the presence of a suitable excess of acid until the lead sulfate has been sufficiently sulfidized, together with the copper, to enable flotation thereof, and finally subjecting the resulting mixture to a flotation treatment; substantially as described. In testimony whereof I affix my signature.

RAYMOND F. BACON.